

## UNITED STATES PATENT OFFICE

2,134,357

## HIGH TRACTIVE RESISTANCE BITUMINOUS SURFACING

Joseph H. Conzelman, Birmingham, Ala., assignor to Alabama Asphaltic Limestone Company, Birmingham, Ala., a corporation of Alabama

No Drawing. Application August 26, 1935,  
Serial No. 37,939

2 Claims. (Cl. 94—23)

This invention relates to a new and novel method of securing a non-skid surface, or high tractive resistance, on bituminous road or street surfaces.

5 Tractive resistance, or the ability to resist skidding, is a much sought for asset in any pavement surfacing. Asphalt pavements, adhesive and resilient when being laid, offer more possibilities for the production of a non-skid riding surface 10 than any other hard-surface type of paving. However, dense, moisture-resisting asphalt mixtures—and these are equally important qualities for they increase the life of the resulting pavement—are popularly supposed to offer less tractive resistance than the open type asphalt mixtures. This has resulted in the use—especially 15 among the cold laid types—of bituminous surfaces high in voids, neglecting almost entirely the established and proven principles of bituminous mixture design. Such mixtures, while possibly 20 low in first cost, are expensive because they are open to deterioration from continued attacks of moisture and the elements and also because they are of little protection against moisture to the 25 base on which they are laid.

Asphalt coated stone, slag or gravel, from  $\frac{3}{4}$ " to  $\frac{1}{4}$ " in size, has been used on dense asphalt pavements to increase tractive resistance. On hot mix pavements these chips coated with from 30 3% to 6% of asphalt have been applied to the surface, after it has been rolled at least once, in the amount of from five to twelve pounds per square yard. When used in these amounts the bituminous coated chips segregate to some extent, for uniform distribution is extremely difficult, and the pockets of chips formed tend to ravel very quickly under traffic affecting adversely the appearance and often the quality of the pavement. The efficiency of the chips in making the 35 pavement more non-skid than it would be without them is also open to question partly because of the size of the chips used and also because in most instances the stone, slag or gravel is of such quality that traffic soon wears it away, or at least wears 40 it down until it makes a smooth surface with the asphalt paving mixture in which it is embedded.

I have found that a fine material, as for instance sand, will when anchored in the surface of a bituminous pavement produce a non-skid surface 45 much more efficient than the asphalt coated chip surface, provided the material is hard enough to withstand the abrasive action of traffic. Sand seal coats mixed with asphalt have been used on asphalt pavements. One instance is the mixed 50 method seal coat used on Warrenite bitulithic

pavements. This seal coat contains about 11% of asphalt and is used in the amount of about forty pounds per square yard. It is essentially a seal coat and a means of protecting and closing the coarse aggregate mixture on which it is laid, for the amount of asphalt used in the seal coat mixture tends to either fill or overfill voids, greatly reducing and in some cases entirely eliminating its non-skid value.

Crushed stone, slag or fine gravel, and in some instances sand, have also been used as a blotter or cover on bituminous paint—or squeegee—coats used to seal old bituminous pavements and in some cases to seal new asphaltic concrete pavement too low in fine aggregate to close up well 10 when rolled. When so used the chips, gravel or sand whip off the pavement surface under traffic and only a portion of the total amount used is taken up by the asphalt flush, or "squeegee", coat. This results in an excess of bituminous material 15 on the surface of the pavement and, even though a fine material such as sand is used, this excess bituminous material tends to make the pavement slippery.

My method of increasing the non-skid quality 20 of bituminous pavements relates to the use of a fine hard material, such as silica sand, coated with an amount of bituminous material small enough to allow the coated non-skid agent to be distributed very lightly and evenly—one particle of 25 the agent thick, preferably—over the surface of either a hot laid or cold laid type of bituminous pavement. The light bituminous coating used is insufficient to allow the coated non-skid agent to bond together and have sufficient adhesion to be 30 used in any thickness over the surface on which it is used. The light bituminous coating merely facilitates the anchoring of the sand paper like 35 agent into the surface of the bituminous pavement.

As an example of the preparation and use of my non-skid surface I would have available, in convenient piles along the length of the bituminous pavement being laid, the necessary amount of the bituminous coated non-skid agent. This material would be made by adding not more than 5% of bituminous material to a hard, fine aggregate. Preferably, I would use 3% of asphalt cutback or asphalt emulsion to coat a medium or coarse sand. The sand should be so graded that it will all pass 50 a  $\frac{3}{8}$ " screen and should contain not more than 30% of particles that would be retained on a 10 mesh sieve, or more than 25% passing a 100 mesh sieve. The sand may be coated in a pug mill mixer, a cylindrical mixer, by hand with shovels, 55

by a spray, or by any other means which allows control of the amount of bituminous material used.

After the bituminous pavement being laid has been rolled at least once the coated sand is spread by brooming, luting, or by mechanical spreader, uniformly over the surface in the amount of approximately one pound per square yard (not to exceed two pounds per square yard) of pavement. A greater amount may be used, but is ineffective because it will be whipped off by traffic, leaving only the small amount anchored in the bituminous paving surface. After the non-skid agent has been applied, rolling of the asphalt surface is completed in the usual manner.

The lightly bitumen-coated non-skid agent is also effective on old smooth bituminous paving. When used on old bituminous paving the old surface would first be painted with a liquefier for the bitumen, such as kerosene. After the liquefier has had sufficient time to slightly soften the surface bitumen, the non-skid agent is applied in a uniform thin coating by means of brooming, luting, or by mechanical spreader. It should then be rolled into the slightly softened surface of the old pavement.

I do not wish the materials used to be confined to those described in the foregoing example. In place of silica sand I might use slag sand, some types of which are dense and hard enough to withstand abrasion, or where commercially available sand made from crushed granite, trap rock, or other extremely hard rock; or, if available,

iron filings, or other finely ground hard metal could be used. Certain crude oils or road oils might be used instead of asphalt emulsion or asphalt cutback; it is also feasible to use heated bituminous cement of either high or low penetration, if the bituminous cement is used in small enough amount so that the resulting mixture when cool will break up readily into its individual bituminous coated particles.

I claim as my invention:

1. A method of increasing the tractive resistance of bituminous paving, consisting of coating a finely graded hard mineral aggregate or metal with less than five (5%) per cent of bituminous material, and applying this mixture directly over the surface of bituminous paving during the period of rolling in an amount of not more than two (2) pounds per square yard.

2. A method of increasing the tractive resistance of a bituminous pavement, consisting of painting the surface with a solvent, then applying a thin coating of hard mineral aggregate or metal in an amount of approximately 1 to not more than 2 pounds per square yard, so graded that it will all pass a three-eighths ( $\frac{3}{8}$ ") inch screen and not more than twenty-five (25%) per cent pass a one hundred (100) mesh sieve, coated with an amount of bituminous material not more than five (5%) per cent small enough so the coated material will not develop sufficient adhesion to bond together itself after it is mixed or set up after it is laid.

JOSEPH H. CONZELMAN.